



US008397792B2

(12) **United States Patent**  
**Kawamoto et al.**

(10) **Patent No.:** **US 8,397,792 B2**  
(45) **Date of Patent:** **Mar. 19, 2013**

(54) **CONTINUOUS CASTING MOLD AND  
CONTINUOUS CASTING METHOD OF  
ROUND BILLET**

(75) Inventors: **Masayuki Kawamoto**, Kashima (JP);  
**Yuichi Tsukaguchi**, Kashima (JP);  
**Masahito Hanao**, Kashima (JP);  
**Atsushi Hirata**, Wakayama (JP);  
**Hiroshi Hayashi**, Wakayama (JP);  
**Manabu Adachi**, Wakayama (JP)

(73) Assignee: **Sumitomo Metal Industries, Ltd.**,  
Osaka (JP)

(\*) Notice: Subject to any disclaimer, the term of this  
patent is extended or adjusted under 35  
U.S.C. 154(b) by 0 days.

(21) Appl. No.: **13/529,262**

(22) Filed: **Jun. 21, 2012**

(65) **Prior Publication Data**

US 2012/0255700 A1 Oct. 11, 2012

**Related U.S. Application Data**

(60) Division of application No. 12/579,495, filed on Oct.  
15, 2009, now Pat. No. 8,225,843, which is a  
continuation of application No. PCT/JP2007/064564,  
filed on Jul. 25, 2007.

(30) **Foreign Application Priority Data**

Jun. 28, 2007 (JP) ..... 2007-170396

(51) **Int. Cl.**  
**B22D 11/08** (2006.01)

(52) **U.S. Cl.** ..... **164/441; 164/447**

(58) **Field of Classification Search** ..... **164/441,  
164/447**

See application file for complete search history.

(56)

**References Cited**

**U.S. PATENT DOCUMENTS**

5,853,043 A 12/1998 Takeuchi et al.

**FOREIGN PATENT DOCUMENTS**

|    |             |         |
|----|-------------|---------|
| JP | 59-165748   | 11/1984 |
| JP | 59-165749   | 11/1984 |
| JP | 132184      | 5/1996  |
| JP | 3022211     | 1/2000  |
| JP | 2003-136203 | 5/2003  |

*Primary Examiner* — Erin Saad

(74) *Attorney, Agent, or Firm* — Clark & Brody

(57) **ABSTRACT**

In a mold for continuously casting a round billet with a curved type continuous casting apparatus, assuming that  $D_0$  (m) is an inner diameter at a lower mold edge and  $R_0$  (m) is a curvature radius of an outer curvature side at the lower mold edge, when a rate of change  $T_p$  (%/m) in mold inner diameter per unit length along a casting direction is expressed by Formula 1, and when a rate of change  $R_p$  (%/m) in curvature radius of an outer curvature side per unit length along the casting direction is expressed by Formula 2, the rate of change  $T_p$  in mold inner diameter and the rate of change  $R_p$  in curvature radius satisfy a relationship expressed by Formula 3;

$$Tp = (1/D_0) \times (dD/dx) \times 100 (\%/m) \quad \text{Formula 1}$$

$$Rp = (1/R_0) \times (dR/dx) \times 100 (\%/m) \quad \text{Formula 2}$$

where  $D$  in Formula 1 is a mold inner diameter at a distance  $x$  away from an upper mold edge and  $R$  in Formula 2 is a curvature radius of the outer curvature side at the distance  $x$ ,

$$Rp = (Tp/2) \times (D_0/R_0) \quad \text{Formula 3}$$

Uniform and good contact is obtained between the billet and a mold inner peripheral surface over a whole circumference, so that the casting-defect-free high-quality round billet can stably be produced.

**3 Claims, 5 Drawing Sheets**



FIG. 1



FIG. 2



FIG. 3



FIG. 4



FIG. 5



## 1

**CONTINUOUS CASTING MOLD AND  
CONTINUOUS CASTING METHOD OF  
ROUND BILLET**

This application is a divisional of U.S. Ser. No. 12/579,495 filed on Oct. 15, 2009, which is a continuation of International Patent Application No. PCT/JP2007/064564, filed Jul. 25, 2007. This PCT application was not in English as published under PCT Article 21(2).

**TECHNICAL FIELD**

The present invention relates to a continuous casting mold used in continuously casting round billets with a curved type continuous casting apparatus and a continuous casting method of round billets in which said continuous casting mold is used.

**BACKGROUND ART**

In continuously casting a round billet having a round shape cross section, compared with the continuous casting of a rectangular billet having a rectangular shape cross section, the billet is unevenly cooled because a mold inner wall (an inner peripheral surface in the case of the round billet mold) is unstably in contact with the billet. When the billet is excessively unevenly cooled, a longitudinal cracking defect is generated in the billet, and a break out is generated due to the longitudinal cracking defect. Therefore, the casting cannot be continued at last.

In order to circumvent the generation of such situation, there have been proposed such various methods that an inner diameter of the mold is decreased according to solidification shrinking, and mold powder fed into the mold are improved during the continuous casting to adjust contact between the mold inner peripheral surface and the billet. For example, Japanese Utility Model Application Publication No. 59 (1984)-165748 proposes a mold, in which an inner diameter is decreased downward and a decrease ratio of the inner diameter is changed in two steps. Further, Japanese Utility Model Application Publication No. 59 (1984)-165749 proposes a mold, in which a tapered surface whose inner diameter is continuously decreased downward and the change in inner diameter is matched with the solidification shrinking. According to the proposed molds, it is said that the uniform contact can be achieved between the mold inner peripheral surface and the billet.

However, in the mold proposed in Japanese Utility Model Application Publication No. 59 (1984)-165748 mentioned above, it is difficult to maintain the good contact between the mold inner peripheral surface and the billet in a whole region from an upper portion to a lower portion of the mold during the continuous casting. Moreover, in the mold proposed in Japanese Utility Model Application Publication No. 59 (1984)-165749 mentioned above, there is a problem in application, although it is possible theoretically that the good contact is maintained between the mold inner peripheral surface and the billet in the whole region from the upper portion to the lower portion of the mold during the continuous casting. That is, a solidification shrinking amount of the billet is difficult to be measured, and it is necessary to change the mold according to each steel grade because the solidification shrinking amount is changed when a chemical composition of steel to be cast is changed, and further, the shrinking amount of casting direction is changed when a casting speed is changed. Accordingly, such proposed molds cannot be used in a commercial operation.

## 2

The applicant has proposed a mold in Japanese Patent No. 3022211, in which the uniform contact is achieved between the mold inner peripheral surface and the billet to perform uniform cooling in continuously casting the round billet. The mold from the upper edge to the lower edge is divided into at least three regions along the casting direction, and the inner diameter of the mold is gradually decreased from the upper edge toward the lower edge by defining a rate of change in mold inner diameter per unit length along the casting direction in each region.

**DISCLOSURE OF THE INVENTION**

However, in the mold proposed in Japanese Patent No. 3022211 mentioned above, although heat transfer between the mold inner peripheral surface and the billet can be homogenized during the continuous casting, a condition on which the expected effect is obtained is restricted. For example, there is a problem that the casting cannot be performed in casting the steel having the different solidification shrinking amount or a problem in changing the casting speed. Particularly, the problem becomes prominent in the case where the inner peripheral surface of the mold is length-wise curved (hereinafter, "curved" generally is used to designate "length-wise curved") according to the shape of the billet like the continuous casting mold which is used to continuously cast the round billet with the curved type continuous casting apparatus.

In view of the foregoing, an object of the present invention is to provide a continuous casting mold which can stably perform the continuous casting of the casting-defect-free round billet and a continuous casting method in which the continuous casting mold is used when the round billet is continuously cast with the curved type continuous casting apparatus.

In order to achieve the object, the present invention provides a mold for continuously casting a round billet with a curved type continuous casting apparatus, the mold having an inner diameter  $D_0$  (m) at a lower edge thereof, and an outer length-wise curvature (hereinafter, "curvature" is generally used to designate "length-wise curvature") surface having a curvature radius  $R_0$  (m) at the lower edge of the mold, and at the same time the round billet continuous casting mold characterized in that, when a rate of change  $T_p$  (%/m) in mold inner diameter per unit length along a casting direction is expressed by Formula 1, and when a rate of change  $R_p$  (%/m) in curvature radius of an outer curvature side per unit length along the casting direction is expressed by Formula 2, the rate of change  $T_p$  in mold inner diameter and the rate of change  $R_p$  in curvature radius satisfy a relationship expressed by Formula 3;

$$T_p = (1/D_0) \times (dD/dx) \times 100(\%/m) \quad \text{Formula 1}$$

where  $D$  is a mold inner diameter at a distance  $x$  away from an upper edge of a cooled mold surface,

$$R_p = (1/R_0) \times (dR/dx) \times 100(\%/m) \quad \text{Formula 2}$$

where  $R$  is a curvature radius of an outer curvature side at a distance  $x$  away from an upper edge of a cooled mold surface, and

$$R_p = (T_p/2) \times (D_0/R_0). \quad \text{Formula 3}$$

In the configuration of the present invention, because a center line of the inner peripheral surface of the mold is aligned with a center line of the billet in continuously casting the round billet, a biased force is not exerted to the billet from the mold and an even force is exerted over the whole circum-

ference, and the uniform and good contact between the billet and the mold inner peripheral surface can be obtained over the whole circumference.

In the round billet continuous casting mold according to the present invention, preferably the mold is divided into three regions along the casting direction, the rate of change  $T_p$  in mold inner diameter ranges from 12 to 16%/m in a first region, the first region being allocated from an upper edge of a cooled mold surface to a zone of 50-100 mm, the cooled mold surface being the side which molten steel is poured to, the zone of 50-100 mm being between the positions of 50 mm and 100 mm away from the upper mold edge, the rate of change  $T_p$  in mold inner diameter continuously varies from 12-16%/m to 0.8-1.4%/m in a second region, the second region successively following the first region and being allocated from said zone of 50-100 mm to a zone of 250-300 mm, the zone of 250-300 mm being between the positions of 250 mm and 300 mm away from the upper mold edge, and the rate of change  $T_p$  in mold inner diameter ranges from 0.8 to 1.4%/m in a third region, the third region successively following the second region and being allocated from said zone of 250-300 mm to the lower edge of the mold.

In the round billet continuous casting mold according to the present invention, the rate of change  $R_p$  in curvature radius ranges from  $6 \times (D_o/R_o)$  to  $8 \times (D_o/R_o)$  (%/m) in a first region, the first region being from the upper edge of the cooled mold surface to the zone of 50-100 mm, the cooled mold surface being the side to which molten steel is poured, the zone of 50-100 mm being between the positions of 50 mm and 100 mm away from the upper mold edge, the rate of change  $R_p$  in curvature radius continuously varies from  $6 \times (D_o/R_o)$ - $8 \times (D_o/R_o)$  (%/m) to  $0.4 \times (D_o/R_o)$ - $0.7 \times (D_o/R_o)$  (%/m) in a second region, the second region successively following the first region and being allocated from said zone of 50-100 mm to a zone of 250-300 mm, the zone of 250-300 mm being between the positions of 250 mm and 300 mm away from the upper mold edge, and the rate of change  $R_p$  in curvature radius ranges from  $0.4 \times (D_o/R_o)$  to  $0.7 \times (D_o/R_o)$  (%/m) in a third region, the third region successively following the second region and being from said zone of 250-300 mm to the lower mold edge, preferably.

Further, in order to achieve the above-mentioned object, a round billet continuous casting method in which the round billet continuous casting mold is used, the round billet continuous casting method is characterized in that continuous casting is performed while a mold powder is being fed onto a surface of the molten steel poured into the continuous casting mold, wherein the mold powder having a viscosity of 0.1 to 1.0 Pa·s at 1573K, a solidification temperature of not less than 1273K, and a mass % ratio of 1.0 to 1.4 in terms of  $(CaO + CaF_2 \times 0.718)/SiO_2$ , a Na content of not more than 5.0 mass % in  $Na_2O$  equivalent, a F concentration of not more than 7.0 mass %, a Mg content of 5-13 mass % in  $MgO$  equivalent, and an Al content of 6-18 mass % in  $Al_2O_3$  equivalent.

According to the round billet continuous casting mold of the invention and the continuous casting method of the present invention in which the mold is used, in the continuous casting with the curved type continuous casting apparatus, the uniform and good contact between the billet and the mold inner peripheral surface is achieved over the whole circumference because the force is evenly exerted to the whole circumference of the billet. As a result, the casting-defect-free high-quality round billet can stably be produced.

#### BRIEF DESCRIPTION OF THE DRAWINGS

FIG. 1 is a vertical cross section showing a frame format of configuration of a conventional round billet continuous casting mold;

FIG. 2 is a vertical cross section showing a frame format of configuration of a round billet continuous casting mold according to the present invention;

FIG. 3 is a vertical cross section for explaining a specific example of the round billet continuous casting mold of the invention;

FIG. 4 is a diagram showing a variation range of a mold copper surface temperature for each casting condition in embodiment; and

FIG. 5 is a diagram showing an index of longitudinal cracking for each casting condition in the embodiment.

#### BEST MODE FOR CARRYING OUT THE INVENTION

15 The inventors studied in detail the problems involved in the conventional mold used in the curved type continuous casting apparatus, and the inventors completed the invention by paying attention to the curvature radius of the mold which the attention has not been given to because of a design standard.

20 FIG. 1 is a vertical cross section showing a frame format of configuration of a conventional round billet continuous casting mold. As shown in FIG. 1, a conventional mold 101 used in the curved type continuous casting apparatus has a constant length-wise curvature radius  $R_o$  of a datum line 101c along the outer length-wise curvature side in the inner peripheral surface. The curvature radius  $R_o$  is substantially matched with the curvature radius of the outer curvature side of a billet 11 withdrawn from the mold 101. A mold inner diameter  $D_o$  at its lower edge 101b is determined according to each diameter of the billet 11.

25 As with the molds proposed in Japanese Utility Model Application Publication No. 59 (1984)-165748, Japanese Utility Model Application Publication No. 59 (1984)-165749, and Japanese Patent No. 3022211, in an inner peripheral surface of the mold 101, the inner diameter of the mold

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465

eter at a lower edge of the mold and  $R_0$  (m) is a curvature radius of an outer curvature side at the lower edge of the mold, when a rate of change  $T_p$  (%/m) in mold inner diameter per unit length along a casting direction is expressed by Formula 1, and when a rate of change  $R_p$  (%/m) in curvature radius of an outer curvature side per unit length along the casting direction is expressed by Formula 2, the rate of change  $T_p$  in mold inner diameter and the rate of change  $R_p$  in curvature radius satisfy a relationship expressed by Formula 3;

$$Tp = (1/D_0) \times (dD/dx) \times 100\%/\text{m} \quad \text{Formula 1}$$

where  $D$  is a mold inner diameter at a distance  $x$  away from an upper edge of a cooled mold surface,

$$Rp = (1/R_0) \times (dR/dx) \times 100\%/\text{m} \quad \text{Formula 2}$$

where  $R$  is a curvature radius of an outer curvature side at a distance  $x$  away from an upper edge of a cooled mold surface, and

$$Rp = (Tp/2) \times (D_0/R_0). \quad \text{Formula 3}$$

FIG. 2 is a vertical cross section showing a frame format of configuration of a round billet continuous casting mold according to the present invention. As shown in FIG. 2, in a mold 1 according to the invention used in the curved type continuous casting apparatus, it is assumed that  $D_0$  is the inner diameter at a lower edge 1b of the mold 1 and  $R_0$  is the curvature radius of a datum line 1c along the outer curvature side in the inner peripheral surface at the lower edge 1b of the mold 1. The mold inner diameter  $D_0$  at the lower edge 1b of the mold is determined according to each diameter of the billet 11 to be cast. The curvature radius  $R_0$  at the lower edge 1b of the mold 1 is substantially matched with the curvature radius of the outer curvature side of the billet 11 withdrawn from the mold 1, which is inherently owned by the applied curved type continuous casting apparatus.

The inner peripheral surface of the mold 1 has a lengthwise tapered shape such that the inner diameter thereof is gradually increased from the lower edge 1b toward the upper edge 1a. At this point, assuming that  $D$  is a mold inner diameter at a distance  $x$  from the upper edge 1a of the cooled mold surface, the rate of change  $T_p$  in mold inner diameter can be expressed by Formula 1. Similarly, assuming that at a distance  $x$  from the upper edge 1a of the cooled mold surface,  $R$  is a curvature radius of the datum line 1c along the outer curvature side, the rate of change  $R_p$  in curvature radius at this position can be expressed by Formula 2. And, the mold inner diameter  $D$  and the curvature radius  $R$  are set at the distance  $x$  away from the upper edge 1a of the cooled mold surface such that at this position, the rate of change  $T_p$  in mold inner diameter and the rate of change  $R_p$  in curvature radius satisfy Formula 3.

When the mold inner diameter  $D$  and the curvature radius  $R$  are set according to the definition of Formula 3, the inner diameter is gradually increased from the lower edge 1b toward the upper edge 1a in the inner peripheral surface of the mold 1 while the increase in inner diameter is evenly distributed to the outer curvature side and the inner curvature side. That is, a center line MC representing a plot of inside diameter centers at elevations ranging from the lower edge 1b and the upper edge 1a is matched with a center line BC of the round billet 11 over the whole region from the lower edge 1b to the upper edge 1a of the mold 1.

The reason why such situation is defined by Formula 3 is as follows. In order to match the center line MC of the mold inner peripheral surface with the center line BC of the billet, it is necessary that the increase in inner diameter of the mold 1 be evenly distributed to the outer curvature side and the inner curvature side while centering around the center line BC of the billet 11. Therefore, it is necessary that a half (1/2) of the rate of change  $T_p$  in mold inner diameter is assigned to the

curvature radius  $R$  of the outer curvature side at the distance  $x$  away from the upper edge 1a of the mold surface. This enables the curvature radius  $R$  of the outer curvature side to be expressed by a following Formula 4 based on the rate of change  $T_p$  in mold inner diameter:

$$R = R_0 + D_0 \times (Tp/2). \quad \text{Formula 4}$$

Similarly, the curvature radius  $R$  of the outer curvature side can be expressed by a following Formula 5 based on the rate of change  $R_p$  in curvature radius:

$$R = R_0 + R_0 \times Rp. \quad \text{Formula 5}$$

Formula 3 can be derived from the relationship between Formula 4 and 5. Therefore, when the relationship expressed by Formula 3 is satisfied, the center line MC of the mold inner peripheral surface is matched with the center line BC of the billet 11.

According to the continuous casting mold of the present invention, in performing the continuous casting of the round billet with the mold, because the center line of the mold inner peripheral surface is matched with the center line of the billet, the mold does not exert the biased force to the billet, and the even force is exerted to the whole circumference of the billet. Therefore, the uniform and good contact between the billet and the mold inner peripheral surface is achieved over the whole circumference, which allows the high-quality round billet to be stably obtained. The same holds true for the case in which the steel having the different solidification shrinking amount is cast or the case in which the casting speed is changed during the casting.

Then, a preferred example of the continuous casting mold of the present invention will be described in the followings.

In the specific example, the continuous casting mold is divided into three regions along the casting direction, the rate of change  $T_p$  in mold inner diameter ranges from 12 to 16%/m in a first region, the first region being allocated from an upper edge of a cooled mold surface to a zone of 50-100 mm, the mold surface being the side which molten steel is poured to, the zone of 50-100 mm being between the positions of 50 mm and 100 mm away from the upper mold edge, the rate of change  $T_p$  in mold inner diameter of continuously varies from 12-16%/m to 0.8-1.4%/m in a second region, the second region successively following the first region and being allocated from said zone of 50-100 mm to a zone of 250-300 mm, the zone of 250-300 mm being between the positions of 250 mm and 300 mm away from the upper mold edge, and the rate of change  $T_p$  in mold inner diameter ranges from 0.8 to 1.4%/m in a third region, the third region successively following the second region and being from said zone of 250-300 mm to the lower edge of the mold. At this point, the rate of change  $R_p$  in curvature radius is determined so as to satisfy the relationship of Formula 3 based on the rate of change  $T_p$  in mold inner diameter.

In other words, the rate of change  $R_p$  in curvature radius ranges from  $6 \times (D_0/R_0)$  to  $8 \times (D_0/R_0)$  (%/m) in a first region, the first region being allocated from an upper edge of a cooled mold surface to a zone of 50-100 mm, the mold surface is the side which molten steel is poured to, the zone of 50-100 mm being between the positions of 50 mm and 100 mm away from the upper mold edge, the rate of change  $R_p$  in curvature radius continuously varies from  $6 \times (D_0/R_0)$ - $8 \times (D_0/R_0)$  (%/m) to  $0.4 \times (D_0/R_0)$ - $0.7 \times (D_0/R_0)$  (%/m) in a second region, the second region successively following the first region and being from said zone of 50-100 mm to a zone of 250-300 mm, the zone of 250-300 mm being between the positions of 250 mm and 300 mm away from the upper mold edge, and the rate of change  $R_p$  in curvature radius ranges from  $0.4 \times (D_0/R_0)$  to  $0.7 \times (D_0/R_0)$  (%/m) in a third region, the third region successively following the second region and being from said zone of 250-300 mm to the lower edge of the mold. At this point,

the rate of change  $T_p$  in mold inner diameter is determined so as to satisfy the relationship of Formula 3 based on the rate of change  $R_p$  in curvature radius.

FIG. 3 is a vertical cross section for explaining a specific example of the round billet continuous casting mold of the invention. For convenience, the tapered inner peripheral surface of the mold is constant and the curved state is not shown in FIG. 3.

As shown in FIG. 3, the mold 1 of the present invention to the lower edge 1b from the upper edge 1a of a cooled mold surface side where molten steel 10 is poured is divided into three regions A1, A2, and A3 along the casting direction. A boundary between the first region A1 and the second region A2 is located within a zone ranging from 50 to 100 mm from the upper edge 1a of the cooled mold surface side, and a boundary between the second region A2 and the third region A3 is located within a zone ranging from 250 to 300 mm from the upper edge 1a of the cooled mold surface. The rate of change  $T_p$  in mold inner diameter is set to 12 to 16%/m in the first region A1, the rate of change  $T_p$  in mold inner diameter is continuously varied from 12-16%/m to 0.8-1.4%/m in the second region A2 which successively follows the first region A1, and the rate of change  $T_p$  in mold inner diameter of the mold is set to 0.8-1.4%/m in the third region A3 which successively follows the second region A2. During the continuous casting, mold powders 12 are fed onto the surface of the molten steel 10 in the mold 1.

The reason why the rate of change  $T_p$  in mold inner diameter is set to the range of 12 to 16%/m in the first region that is allocated from the upper mold edge to the zone of 50-100 mm is that the first region is used to effectively achieve the uniform contact between the mold inner peripheral surface and the billet. That is, when the first region is shorter than 50 mm, the shrinking of the mold becomes smaller than the shrinking of the solidified shell, which causes the non-uniform contact to generate longitudinal cracking. On the other hand, when the first region is longer than 100 mm, the shrinking of the mold becomes excessively large to generate constraint due to the seizure between the mold and billet. The constraint is generated when the rate of change  $T_p$  in mold inner diameter is excessively larger than a specified value, and the longitudinal cracking is generated when the rate of change  $T_p$  in mold inner diameter of the mold is excessively smaller than the specified value.

The reason why the rate of change  $T_p$  in mold inner diameter is continuously varied from 12-16%/m to 0.8-1.4%/m in the second region that is allocated next to the first region and from said zone of 50-100 mm to the zone of 250-300 mm, is that when the second region is shorter than the range determined by the datum point of 250 mm, the shrinking of the mold becomes smaller than the shrinking of the solidified shell, which causes the non-uniform contact to generate longitudinal cracking. On the other hand, when the second region is longer than the range determined by the datum point of 300 mm, the shrinking of the mold becomes excessively large to generate constraint due to the seizure between the mold and the billet. The seizure-related constraint is generated when the rate of change  $T_p$  in mold inner diameter is excessively larger than the specified value, and the longitudinal cracking is generated when the rate of change  $T_p$  in mold inner diameter is excessively smaller than the specified value. Further, in the third region between the end of the second region and the lower mold edge, it is for the same reason that the rate of change  $T_p$  in mold inner diameter is set to the range of 0.8 to 1.4%/m.

The use of the continuous casting mold of the specific example can achieve the better contact between the billet and

the mold inner peripheral surface to obtain the high-quality round billet. As for the mold powder which constitutes a heat transfer medium between the mold inner peripheral surface and the billet, a material having the following physical properties and composition is used in the mold of the present invention, which allows the higher-quality round billet to be obtained compared with the use of the conventional mold powder.

The mold powder having the following physical properties and composition can be used in the round billet continuous casting mold of the invention. That is, a viscosity of 0.1 to 1.0 Pa·s at 1573K, a solidification temperature of not less than 1273K, and a mass % ratio of 1.0 to 1.4 in terms of  $((\text{CaO} + \text{CaF}_2 \times 0.718)/\text{SiO}_2)$ , a Na content of not more than 5.0 mass % in  $\text{Na}_2\text{O}$  equivalent, a F concentration of not more than 7.0 mass %, a Mg content of 5 to 13 mass % in  $\text{MgO}$  equivalent, and an Al content of 6 to 18 mass % in  $\text{Al}_2\text{O}_3$  equivalent. Table 1 shows the physical properties and composition of the mold powder.

TABLE 1

|                                                                                    |                    |
|------------------------------------------------------------------------------------|--------------------|
| Viscosity at 1573K                                                                 | 0.1 to 1.0 Pa·s    |
| Solidification temperature                                                         | 1273K or more      |
| Mass % ratio in terms of $((\text{CaO} + \text{CaF}_2 \times 0.718)/\text{SiO}_2)$ | 1.0 to 1.4         |
| Na content in $\text{Na}_2\text{O}$ equivalent                                     | 5.0 mass % or less |
| F concentration                                                                    | 7.0 mass % or less |
| Mg content in $\text{MgO}$ equivalent                                              | 5 to 13 mass %     |
| Al content in $\text{Al}_2\text{O}_3$ equivalent                                   | 6 to 18 mass %     |

(Note)

\*Solidification temperature expresses a temperature at which viscosity rises rapidly in viscosity measurement.

\*Because usually a cationic concentration is determined in a chemical analysis value, the content is defined by converting the chemical analysis value into a concentration in oxide equivalent.

\*For  $\text{CaO}$ , the value is expressed by converting a Ca concentration into a  $\text{CaO}$  concentration.

In the mold powder, when the viscosity at 1573K is lower than 0.1 (Pa·s), the powder is non-uniformly poured between the mold inner peripheral surface and the billet, and the heat is non-uniformly dissipated. This causes the generation of the longitudinal cracking or seizure-related constraint and/or the defect by migrating the powder into molten steel. On the other hand, when the viscosity is more than 1.0 Pa·s, the lack of the inflow of the powder between the mold inner peripheral surface and the billet causes the generation of the seizure-related constraint.

When the solidification temperature is lower than 1273K, a liquid phase of the powder is increased between the mold inner peripheral surface and the billet, and the cooling is excessively provided. Therefore, the billet is distorted by a thermal stress to generate the longitudinal cracking.

When the mass % ratio in terms of  $((\text{CaO} + \text{CaF}_2 \times 0.718)/\text{SiO}_2)$  is lower than 1.0,  $\text{SiO}_2$  in the powder oxidizes Mn in the molten steel to change the composition, and the defect is generated in the billet surface. And when the Mg content in  $\text{MgO}$  equivalent is lower than 5 mass %, because crystallization is not stabilized, the cooling is excessively provided to generate the longitudinal cracking. On the other hand, when the mass % ratio in terms of  $((\text{CaO} + \text{CaF}_2 \times 0.718)/\text{SiO}_2)$  is more than 1.4, or when the Mg content in  $\text{MgO}$  equivalent is more than 13 mass %, the powder film is excessively shrunk, and the good contact is disturbed between the billet and the mold inner peripheral surface to generate the longitudinal cracking, or the powder is not melted because the solidification temperature is associated to become excessively high.

When the Na content in  $\text{Na}_2\text{O}$  equivalent is more than 5.0 mass %, or when F concentration is more than 7.0 mass %, a melting behavior of the powder becomes defective to generate an entrapment defect, etc.

When the Al content in  $\text{Al}_2\text{O}_3$  equivalent is less than 6 mass %, the composition of the crystal is changed during the

casting to non-uniformly provide the cooling. On the other hand, when the Al content in  $\text{Al}_2\text{O}_3$  equivalent is more than 18 mass %, the powder is hardly flowed inbetween the billet and the mold inner peripheral surface because the solidification temperature is associated to become excessively high.

Accordingly, the round billet having the better quality can be produced, when the continuous casting is performed while the mold powder having the physical properties and composition defined as described above is fed onto the surface of the molten steel in the mold of the present invention.

## EXAMPLES

Tests were performed with a curved type continuous casting apparatus which has an one-point straightening device in order to confirm the effects of the mold of the present invention and the continuous casting method in which the mold was used. The curved type continuous casting apparatus which has an one-point straightening device had the curvature radius ( $R_0$ ) of 10 m. The steels having C ranging from 0.06 to 0.35 mass % and Mn ranging from 0.8 to 1.8 mass % were used in the test of the embodiment. Although it is not always necessary to contain Cr, Cr is set to less than 3 mass % when Cr is

contained. The casting tests were performed with three steel grades A, B, and C shown in Table 2.

TABLE 2

| 5     | Steel | Chemical composition (mass %) |      |      |        |        |      |       |
|-------|-------|-------------------------------|------|------|--------|--------|------|-------|
|       |       | Balance: Fe and impurities    |      |      |        |        |      |       |
| grade | C     | Mn                            | Si   | P    | S      | Cr     | Al   |       |
| 10    | A     | 0.27                          | 0.41 | 0.26 | 0.0080 | 0.0030 | 0.97 | 0.035 |
|       | B     | 0.23                          | 1.29 | 0.30 | 0.0110 | 0.0060 | 0.46 | 0.025 |
|       | C     | 0.22                          | 0.61 | 0.18 | 0.0220 | 0.0060 | —    | 0.018 |

(Note)  
“—” shows that the element is not contained.

15 In the embodiment, the molten steel was poured into molds M1 to M20 (having the inner diameter ( $D_0$ ) of 225 mm at the lower edge of the mold and the length of 900 mm) shown in Table 3, mold powder P1 to P11 shown in Table 4 was fed onto the surface of the molten steel, and the continuous casting was  
20 performed at a casting speed of 2.0 m/min. Table 5 shows casting conditions A to AF which are in combination of the steel grades A to C, the molds M1 to M20, and the powder P1 to P11 in the embodiment.

TABLE 3

TABLE 3-continued

|              |                                                             |       |       |       |       |       |       |       |     |     |     |
|--------------|-------------------------------------------------------------|-------|-------|-------|-------|-------|-------|-------|-----|-----|-----|
| Third region | Rate of change in mold inner diameter in third region (%/m) | 1.1   | 1.1   | 1.1   | 1.1   | 1.1   | 0.8   | 1.4   | 1.1 | 0.8 | 1.4 |
|              | Rate of change in curvature radius in first region (%/m)    | 0.135 | 0.180 | 0.158 | 0.158 | 0.158 | 0.158 | 0.158 | 0*  | 0*  | 0*  |
|              | Rate of change in curvature radius in third region (%/m)    | 0.012 | 0.012 | 0.012 | 0.012 | 0.012 | 0.009 | 0.016 | 0*  | 0*  | 0*  |
|              | Rate of change in mold inner diameter (%/m)                 | 1.1   | 1.1   | 1.1   | 1.1   | 1.1   | 0.8   | 1.4   | 1.1 | 0.8 | 1.4 |
|              | Rate of change in curvature radius (%/m)                    | 0.012 | 0.012 | 0.012 | 0.012 | 0.012 | 0.009 | 0.016 | 0*  | 0*  | 0*  |
|              | Classification                                              | I     | I     | I     | I     | I     | I     | I     | C   | C   | C   |
|              |                                                             |       |       |       |       |       |       |       |     |     |     |

(Note)

In classification, "I" means Inventive example and "C" means Comparative example.

\*shows that the numerical data deviates from the range defined in the present invention.

TABLE 4

|                                         | P1   | P2   | P3   | P4    | P5    | P6   | P7   | P8   | P9   | P10  | P11  |
|-----------------------------------------|------|------|------|-------|-------|------|------|------|------|------|------|
| Viscosity (Pa <sup>-s</sup> )           | 0.50 | 0.40 | 0.60 | 0.40  | 0.60  | 0.35 | 0.36 | 0.49 | 0.52 | 0.48 | 0.53 |
| Solidification temperature (K)          | 1505 | 1512 | 1495 | 1600  | 1460  | 1465 | 1463 | 1505 | 1520 | 1500 | 1520 |
| Basicity (—)                            | 1.20 | 1.40 | 1.00 | 1.45* | 0.95* | 1.20 | 1.20 | 1.20 | 1.20 | 1.20 | 1.20 |
| Na <sub>2</sub> O (mass %)              | 0.5  | 0.5  | 0.5  | 0.5   | 0.5   | 6.0* | 0.5  | 4.0  | 2.0  | 4.0  | 4.0  |
| F (mass %)                              | 4.0  | 4.0  | 4.0  | 4.0   | 4.0   | 4.0  | 8.0* | 4.0  | 4.0  | 4.0  | 4.0  |
| MgO (mass %)                            | 8.0  | 8.0  | 8.0  | 8.0   | 8.0   | 8.0  | 8.0  | 6.0  | 13.0 | 8.0  | 8.0  |
| Al <sub>2</sub> O <sub>3</sub> (mass %) | 11.0 | 11.0 | 11.0 | 11.0  | 11.0  | 11.0 | 11.0 | 11.0 | 11.0 | 7.0  | 18.0 |
| Classification                          | I    | I    | I    | C     | C     | C    | C    | I    | I    | I    | I    |

(Note)

Basicity means the mass ratio of (CaO + CaF<sub>2</sub> × 0.718)/SiO<sub>2</sub>.

In classification, "I" means Inventive example and "C" means Comparative example.

\*shows that the numerical data deviates from the range defined in the present invention.

TABLE 5

|                   | Casting condition |     |     |     |     |     |      |      |      |     |     |
|-------------------|-------------------|-----|-----|-----|-----|-----|------|------|------|-----|-----|
|                   | A                 | B   | C   | D   | E   | F   | G    | H    | I    | J   | K   |
| Steel grade       | A                 | A   | A   | A   | A   | A   | A    | A    | A    | A   | A   |
| Mold              | M11*              | M2* | M3* | M4* | M5* | M6* | M7*  | M8*  | M9   | M10 | M11 |
| Mold powder       | P1                | P1  | P1  | P1  | P1  | P1  | P1   | P1   | P1   | P1  | P1  |
| Classification    | C                 | C   | C   | C   | C   | C   | C    | I    | I    | I   | I   |
| Casting condition |                   |     |     |     |     |     |      |      |      |     |     |
|                   | L                 | M   | N   | O   | P   | Q   | R    | S    | T    | U   | V   |
| Steel grade       | A                 | A   | A   | A   | A   | A   | A    | A    | A    | A   | A   |
| Mold              | M12               | M13 | M14 | M15 | M16 | M17 | M18* | M19* | M20* | M15 | M15 |
| Mold powder       | P1                | P1  | P1  | P1  | P1  | P1  | P1   | P1   | P1   | P2  | P3  |
| Classification    | I                 | I   | I   | I   | I   | C   | C    | C    | I    | I   | I   |
| Casting condition |                   |     |     |     |     |     |      |      |      |     |     |
|                   | W                 | X   | Y   | Z   | AA  | AB  | AC   | AD   | AE   | AF  |     |
| Steel grade       | A                 | A   | A   | A   | A   | A   | A    | A    | B    | C   |     |
| Mold              | M15               | M15 | M15 | M15 | M15 | M15 | M15  | M15  | M15  | M15 |     |
| Mold powder       | P4*               | P5* | P6* | P7* | P8  | P9  | P10  | P11  | P1   | P1  |     |
| Classification    | C                 | C   | C   | C   | I   | I   | I    | I    | I    | I   |     |

(Note) In classification,

"I" means Inventive example and "C" means Comparative example.

\*shows that the numerical data deviates from the range defined in the present invention.

The test result was evaluated by a variation range in mold copper surface temperature representing how is the contact between the mold inner peripheral surface and the billet, an index of the longitudinal cracking, and the presence or absence of a withdrawal-disabled accident.

FIG. 4 is a diagram showing a variation range of a mold copper surface temperature for each casting condition in the embodiment. The mold temperature variation range of FIG. 4 shows an effective value (numeric integration average) of the temperature variation of a thermocouple disposed 150 mm away from the upper edge of the mold surface. The thermocouple was disposed inside by 15 mm from the copper surface.

FIG. 5 is a diagram showing an index of longitudinal cracking for each casting condition in the embodiment. The index of longitudinal cracking in FIG. 5 is a cracking length per unit length of the billet.

As is clear from FIGS. 4 and 5, for the casting conditions I to Q, U, V, and AA to AF of the inventive example, the variation in mold copper surface temperature fell well within a tolerable range causing no problem, and the longitudinal cracking was hardly generated. Additionally, a break out or an alarm of seizure-related constraint was not caused.

On the contrary, for the casting conditions A, C, E, F, R to T, and W to Z of the comparative example, the mold copper surface temperature exhibited a large variation which is of an issue in the commercial operation, and the large longitudinal cracking was generated. Among others, the powder P4, P5, P6, and P7 which were of the comparative example were used in the casting conditions W, X, Y, and Z, and the improper mold powder generated the large variation in copper surface temperature. For the casting conditions R, S, and T in which the molds M18, M19, and M20 as being the comparative example were used, and although the rate of change in mold inner diameter was within the proper range, the rate of change in the curvature radius of the casting apparatus was out of the proper range. Therefore, the uniform contact was not maintained between the billet and the mold inner peripheral surface.

For the casting conditions B, D, G, and H as being the comparative example, although the copper surface temperature exhibits the small variation, the molds M1, M4, M7, and M8 as being the comparative example were used. Therefore, the withdrawal-disabled accident was occurred because the rate of change in mold inner diameter was out of the proper range.

#### INDUSTRIAL APPLICABILITY

According to the round billet continuous casting mold of the present invention and the continuous casting method in which said mold is used, in continuously casting the round billet with the curved type continuous casting apparatus, the even force is exerted to the whole circumference of the billet, and the uniform and good contact between the billet and the mold inner peripheral surface is achieved over the whole circumference, so that the casting-defect-free high-quality round billet can stably be produced. Accordingly, the present invention is extremely useful in the continuous casting mold and the continuous casting method in which the high-quality round billet can be produced with the curved type continuous casting apparatus.

What is claimed is:

1. A round billet continuous casting method in which a round billet continuous casting mold is used, the round billet continuous casting mold having an upper edge, a lower edge, and a cooled mold surface extending between the upper and lower edges, the mold also having an inner diameter  $D_o$  (m) at the lower edge thereof, and an outer curvature side thereof is configured to have a curvature radius  $R_o$  (m) at the lower edge thereof, wherein D is a mold inner diameter at a distance x away from the upper edge of the cooled mold surface and  $dD/dx$  represents a change in D with respect to a change in x, and R is a curvature radius of an outer curvature side at a distance x away from the upper edge of the cooled mold surface and  $dR/dx$  represents a change in R with respect to the change in x,

the mold being characterized in that:

given that a rate of change  $T_p$  (%/m) in mold inner diameter per unit length along a casting direction is expressed by Formula 1, and a rate of change  $R_p$  (%/m) in curvature radius of an outer curvature side per unit length along the casting direction is expressed by Formula 2, the rate of change  $T_p$  in mold inner diameter and the rate of change  $R_p$  in curvature radius satisfy a relationship expressed by Formula 3;

$$T_p = (1/D_o) \times (dD/dx) \times 100(\%/m), \quad \text{Formula 1}$$

$$R_p = (1/R_o) \times (dR/dx) \times 100(\%/m), \quad \text{Formula 2}$$

$$R_p = (T_p/2) \times (D_o/R_o); \quad \text{Formula 3}$$

wherein the method comprises feeding a mold powder onto a surface of a molten steel while pouring the molten steel into the continuous casting mold, the mold powder having a viscosity of 0.1 to 1.0 Pa·s at 1573K, a solidification temperature of not less than 1273K, and a mass % ratio of 1.0 to 1.4 in terms of  $(\text{CaO} + \text{CaF}_2 \times 0.718)/\text{SiO}_2$ , a Na content of not more than 5.0 mass % in  $\text{Na}_2\text{O}$  equivalent, a F concentration of not more than 7.0 mass %, a Mg content of 5 to 13 mass % in  $\text{MgO}$  equivalent, and an Al content of 6 to 18 mass % in  $\text{Al}_2\text{O}_3$  equivalent.

2. The method according to claim 1, wherein the mold is divided into three regions along a casting direction, the rate of change  $T_p$  in mold inner diameter ranges from 12 to 16%/m in a first region, the first region being allocated from an upper edge of a cooled mold surface to a zone of 50-100 mm, the cooled mold surface being the side which molten steel is poured to, the zone of 50-100 mm being between the positions of 50 mm and 100 mm away from the upper mold edge, the rate of change  $T_p$  in mold inner diameter continuously varies from 12-16%/m to 0.8-1.4%/m in a second region, the second region successively following the first region and being allocated from said zone of 50-100 mm to a zone of 250-300 mm, the zone of 250-300 mm being between the positions of 250 mm and 300 mm away from the upper mold edge, and the rate of change  $T_p$  in mold inner diameter ranges from 0.8 to 1.4%/m in a third region, the third region successively following the second region and being allocated from said zone of 250-300 mm to the lower mold edge.

3. The method according to claim 1, wherein the mold is divided into three regions along the casting direction, the rate of change  $R_p$  in curvature radius ranges from  $6 \times (D_o/R_o)$  to  $8 \times (D_o/R_o)$  (%/m) in a first region, the first region being allocated from an upper edge of a cooled mold surface to a zone of 50-100 mm, the cooled mold surface being the side which molten steel is poured to, the zone of 50-100 mm being between the positions of 50 mm and 100 mm away from the upper mold edge, the rate of change  $R_p$  in curvature radius

**15**

continuously varies from  $6 \times (D_o/R_o) - 8 \times (D_o/R_o)(\%/\text{m})$  to  $0.4 \times (D_o/R_o) - 0.7 \times (D_o/R_o)(\%/\text{m})$  in a second region, the second region successively following the first region and being allocated from said zone of 50-100 mm to a zone of 250-300 mm, the zone of 250-300 mm being between the positions of 250 mm and 300 mm away from the upper mold edge, and the

5

**16**

rate of change  $R_p$  in curvature radius ranges from  $0.4 \times (D_o/R_o)$  to  $0.7 \times (D_o/R_o)(\%/\text{m})$  in a third region, the third region successively following the second region and being allocated from said zone of 250-300 mm to the lower mold edge.

\* \* \* \* \*

UNITED STATES PATENT AND TRADEMARK OFFICE  
**CERTIFICATE OF CORRECTION**

PATENT NO. : 8,397,792 B2  
APPLICATION NO. : 13/529262  
DATED : March 19, 2013  
INVENTOR(S) : Kawamoto et al.

Page 1 of 1

It is certified that error appears in the above-identified patent and that said Letters Patent is hereby corrected as shown below:

In the Claims:

Column 14, Line 35

ratio of 1.0 to 1.4 in terms of  $(\text{CaO} + \text{CaF}_2 \times 0.718) / \text{SiO}_2$

should read:

ratio of 1.0 to 1.4 in terms of  $((\text{CaO} + \text{CaF}_2 \times 0.718) / \text{SiO}_2)$

Signed and Sealed this  
Twenty-fourth Day of September, 2013



Teresa Stanek Rea  
Deputy Director of the United States Patent and Trademark Office